

H. LUCKENBACH.  
METHOD OF MAKING STRUCTURES FOR SUPERHEATING AND OTHER PURPOSES.  
APPLICATION FILED APR. 26, 1911.

1,025,817.

Patented May 7, 1912.

*Fig. 1.*



*Fig. 2.*



*Fig. 3.*



Witnesses.

D.W. Edelin.

Fred A. Klinge.

Inventor:

H. Luckenbach

by H. Luckenbach, Atty.

# UNITED STATES PATENT OFFICE.

HARRY LUCKENBACH, OF CHICAGO, ILLINOIS, ASSIGNOR, BY MESNE ASSIGNMENTS, TO LUCKENBACH INVENTIONS DEVELOPMENT COMPANY, OF NEW YORK, N. Y., A CORPORATION OF NEW YORK.

## METHOD OF MAKING STRUCTURES FOR SUPERHEATING AND OTHER PURPOSES.

1,025,817.

Specification of Letters Patent.

Patented May 7, 1912.

Application filed April 26, 1911. Serial No. 623,471.

To all whom it may concern:

Be it known that I, HARRY LUCKENBACH, a citizen of the United States, residing at Chicago, in the county of Cook and State of Illinois, have invented certain new and useful Improvements in Methods of Making Structures for Superheating and other Purposes; and I do declare the following to be a full, clear, and exact description of the invention, such as will enable others skilled in the art to which it appertains to make and use the same, reference being had to the accompanying drawings, and to the letters and figures of reference marked thereon, which form a part of this specification.

My invention relates to a method of making structures designed for heating or superheating steam, air or other gases and liquids and for other purposes, and more particularly to such structures in which the channel or chamber for the fluid or agent to be heated is incased or inclosed within a body of metal which serves as a protecting incasement for the chamber or channel to which the fluid is supplied and also serves to absorb and transmit heat to the chamber or channel in which water is to be heated or its heat retained or maintained, or the steam, air or other gases superheated.

The invention has for its object the practice of a method by which the metal chamber or channel of the product is protected against injury or deterioration by heat while casting about it a metal incasement, and by which method also there is provided a granular non-fusible filling confined between the metal chamber or channel and the metal casement cast about it so that the chamber or channel will be protected against injury from the intense heat to which the inclosing incasement may be subjected for the purpose of superheating the fluid or gas passing through the chamber or channel and which also makes it possible to maintain in the chamber or channel such a temperature that the heated air or fluid or gas introduced therein will not lose, or be lowered, in temperature, and thus by maintaining its temperature making it possible to more quickly superheat the same and to bring it to a higher degree of superheat; said granular filling also permitting expansion and contraction of the metal of the chamber or channel.

To the accomplishment of the foregoing and such other objects as may be hereinafter made to appear the invention contemplates the application to the surface of the chamber or channel of a non-fusible plastic composition having the characteristic of retaining its homogeneity without fracture or the formation of fissures during the step of being baked to hardness preparatory to being incased in a body of molten cast metal, and possessing the further characteristic of becoming comminuted or pulverized upon the application of the body of molten cast metal thereto. It is necessary that the plastic composition should not fracture or fissure before the application of the body of molten cast metal to it because if it did, the molten cast metal would come in contact with the wall of the chamber or channel, the same being ordinarily of cast, wrought or steel metal, and disintegrate or destroy the integrity of the material composing the wall of the chamber or channel, and it is also desirable to have the plastic material comminute or pulverize upon the application thereto of the body of molten cast metal so that as the cast, wrought iron, or steel chamber or channel thus becomes incased within a body of cast metal the pulverized non-fusible substance between the wall of the chamber or channel and the body of cast metal will serve to protect the chamber or channel from the destructive influence of the intense heat derived by the cast metal from the heat products of a combustion chamber and transmitted through such body to the chamber or channel containing the fluid or agent to be heated, said pulverized non-fusible substance also permitting expansion and contraction of the metal constituting the chamber or channel which would not be provided for if the non-fusible substance between the body of cast metal and the wall of the chamber or channel were solid. The structure produced comprises a chamber or channel containing the agent to be heated or superheated and the incasing body of cast metal with the non-fusible fire-resisting pulverized substance intervening between the cast metal body and the chamber or channel for the agent or fluid to be acted upon and is susceptible of a diversity of applications or uses where a structure having the characteristics men-

tioned is desirable or necessary for accomplishment of the objects in view. This structure however is not claimed herein as it forms the subject of a separate application, although for clearness in describing the method reference is made to features of the structure and to the accompanying drawing, in which:

Figure 1 represents a coil of pipe incased 10 in a non-fusible fire-resisting coating preparatory to applying thereto a body of molten cast metal; Fig. 2 is a perspective view of a cast iron block having the chamber or pipe incased therein and with the intervening comminuted or pulverized non-fusible filling or substance; and Fig. 3 a section of a cast iron block with inclosed pipe or chamber and intermediate pulverized substance, and curved to represent a section of a 20 fire-box or combustion chamber.

For the purpose of obtaining a proper plastic composition possessing the necessary conditions or characteristics for successfully carrying into effect the invention I have 25 made numerous experiments with a number of different refractory or fire-resisting clays and discovered that many of the materials experimented with failed to give the results because the substance or composition al- 30 though non-fusible would, upon being baked or hardened, crack or have fissures formed therein so that when molten cast metal was applied to the coating the molten metal would find its way through the fis- 35 sures or cracks and coming in contact with the cast or wrought iron or steel chamber or channel would disintegrate or destroy the texture or fiber of the metal so that the chamber or channel would be rendered unfit 40 for the purposes contemplated. Finally I discovered that the non-fusible clay known as "blast furnace clay" is sufficiently moisture receptive as to amalgamate advanta- 45 geously with graphite and a non-inflammable oil so as to form a plastic composition which will adhere tenaciously to the surface of the cast, wrought or steel metal chamber or channel to which applied and enable the same to be baked or hardened 50 without contracting to a degree that would cause fissures or fractures in the plastic coating, thus making it possible to apply molten cast metal to the chamber or channel and this coating without coming in contact with 55 and injuring the metal constituting the chamber or channel.

I obtained the best results by combining with the "blast furnace clay," pulverized graphite in the proportion substantially of 60 one part of pulverized graphite to two parts of the "blast furnace clay" and adding sufficient oil to moisten the mixture and produce a plastic composition which would adhere tenaciously to the iron surface coated 65 with it. I also discovered that by using cot-

ton-seed oil as the moistening agent the best results were obtained because this oil would not inflame or burn under the heat to which the plastic composition and chamber or channel which it inclosed was subjected in 70 the baking or hardening of the composition, but such oil would evaporate thus leaving the composition a hard and solid mass inclosing the metal chamber or channel.

In using this plastic composition I usually apply it to the metal surface 1 to produce a coating 2 varying from one-quarter of an inch to one inch in thickness, and after so coating the metal chamber or channel the whole is placed within a suitable 80 oven for heating and baking the composition until it becomes hard or solid. After the plastic composition has thus been hardened the chamber or channel coated therewith is placed in a suitable mold and molten 85 cast metal, preferably high-grade cast iron, is introduced or applied so as to wholly incase the cast, wrought iron or steel chamber or channel. This molten cast iron coming in contact with the plastic coating disintegrates or comminutes the composition and leaves the same in the condition of a pulverized substance 3 filling the space between the molten cast iron body 4 and the cast, wrought or steel metal chamber or 90 channel, the plastic composition preventing the molten metal from coming in contact with the wrought iron during the molding operation, and the plastic composition when pulverized serving to practically fill the 95 space between the body of cast iron and the cast, wrought iron or steel chamber or channel but allowing of contraction and expansion of the cast, wrought iron or steel 100 chamber or channel in the uses to which the 105 structure may be applied because of the pulverized character of the material lying between the outside cast metal body and the inclosed cast, wrought iron or steel chamber or channel. This non-fusible pulverized 110 material thus interposed between the cast metal body and the cast, wrought iron or steel chamber or channel allows the intense heat to which the cast metal body may be subjected to be transmitted from the cast 115 metal body and through the pulverized filling to the cast, wrought iron or steel chamber or channel without the cast metal body being in direct contact with the surface of the cast, wrought or steel metal chamber or 120 channel. The cast iron body can be subjected to a very high degree of heat which would disintegrate or destroy the cast, wrought iron or steel chamber or channel if allowed to come in direct contact there- 125 with.

It has been proposed heretofore to incase wrought iron pipes in a molten body of cast metal but when molten cast metal is brought in direct contact with a wrought iron pipe 130

the molten metal tends to melt the pipe with which it comes in contact, and I have also learned that if the wrought iron be first coated with a plastic composition that 5 said composition will crack or fracture when dried and when such is the case and molten metal is poured or molded upon the pipe so coated the metal will at once flow through the fracture and coming in contact with the 10 wrought iron will melt or seriously injure the strength of the metal and thus produce a defective structure. But by providing a composition such as I have mentioned these difficulties are overcome and the advantages 15 I have specified are obtained. The "blast furnace clay" forming a part of my composition is a red clay containing a relatively large percentage of magnesia and is commonly used in connection with blast furnaces, and from all my experiments I have 20 found the best results obtained when this "blast furnace clay" is combined with graphite and with oil, particularly cotton-seed oil.

25 The structure produced under the method described is particularly well adapted for use in superheating steam, air or other gases as the cast metal body will without detriment to its texture receive a very high 30 degree of heat and can be brought to a state of incandescence so as to transmit to the cast, wrought iron or steel chamber or channel such a high temperature as to obtain the highest superheating of the steam, air or 35 other gases passing through the cast, wrought iron or steel chamber or channel. It can however also be employed to advantage where water is to be heated by passing it through the cast, wrought iron or steel 40 chamber or channel.

Having described my invention and set forth its merits what I claim is:

1. The method of protecting a hollow

metal channel or chamber from injury by heat consisting in coating the metal chamber or channel with a plastic consisting of non-fusible material, graphite and an oil; then baking the plastic coating, and then incasing the metal channel or chamber and coating in a body of molten metal. 45

2. The method of protecting a hollow metal chamber or channel from injury by heat consisting in coating the metal channel or chamber with a plastic consisting of blast furnace clay, graphite and cotton-seed 50 oil; then baking the plastic coating, and then incasing the channel or chamber and coating in a body of molten cast iron. 55

3. The method of protecting a metal chamber or channel from injury by heat 60 consisting in coating the metal chamber or channel with a plastic consisting of blast furnace clay, graphite and a non-inflammable oil, such as cotton-seed oil; then baking the plastic coating; and then applying 65 a body of molten cast metal to the chamber or channel and coating to granulate or disintegrate the coating and confine it between the chamber or channel and incasing body of cast metal. 70

4. The method of protecting a metal chamber or channel against injury by heat 75 consisting in coating the metal chamber or channel with a non-fusible disintegrable plastic, and then applying a body of molten cast metal to the metal chamber or channel and the plastic composition to granulate or disintegrate the plastic and confine it between the chamber or channel and incasing body of cast metal. 80

In testimony whereof I affix my signature in presence of two witnesses.

HARRY LUCKENBACH.

Witnesses:

EDGAR M. JENNINGS,  
JAMES MIDDLETON.